

Dec. 27, 1927.

1,654,462

A. HORTEN

METHOD OF AND APPARATUS FOR MANUFACTURING CONCRETE PIPES

Filed Feb. 19, 1926



*Fig. 2.*



*Fig. 3.*



*Fig. 6. a*



*Fig. 4.*



A. Morten  
INVENTOR

By: Marks & Clark  
Atlys

## UNITED STATES PATENT OFFICE.

ALPHONS HORTEN, OF BERLIN-WILMERSDORF, GERMANY.

## METHOD OF AND APPARATUS FOR MANUFACTURING CONCRETE PIPES.

Application filed February 19, 1926, Serial No. 89,483, and in Germany February 23, 1925.

My invention relates to improvements in the method of and apparatus for manufacturing concrete pipes such as are used for conducting liquids and gases. My improved 5 method may be used for manufacturing reinforced concrete pipes having a very smooth inner surface.

One of the objects of the improvements is to provide a method by means of which pipes 10 are produced which are free of fine cracks interfering with the strength of the pipe and causing leakage of the fluid. With this object in view my invention consists in manufacturing the wall of the pipe in different 15 layers, one layer being first applied to a suitable core by flinging or squirting soft concrete onto a rotary core, allowing the said concrete to set, and thereafter flinging or squirting another layer of soft concrete onto 20 the inner layer previously produced on the core. Ordinarily each layer has a thickness substantially equal to one half the desired 25 thickness of the wall of the pipe. In the manufacture of re-inforced concrete pipes I place re-inforcing iron in the form of a net or a coil of wire or strip iron on the surface of the set inner layer, and I apply the second or outer layer on the said re-inforcing iron and the inner layer.

30 For economical reasons, and more particularly when manufacturing the pipe in two layers, it is important that the setting of the concrete be completed within a short period of time in order that the cores the cost of 35 which is comparatively high may be used for manufacturing further pipes. Further it is important to carry out the method in such a way that the inner surface of the inner layer be as smooth as possible and that the core 40 can readily be removed from the said pipe. Therefore my method includes a step in which the concrete is rapidly set and it makes use of cores insuring a smooth inner surface of the complete pipe.

45 In my improved method the concrete is flung or squirted on a solid, cylindrical or slightly tapering core made from a material having a high conductivity for heat. After applying the first layer of concrete to the 50 core the concrete is externally heated at a temperature causing rapid setting. In a similar way the second layer of concrete is heated at a suitable temperature. Finally, 55 after the whole mass of concrete has set heating is continued at the outside of the pipe, while a cooling medium is applied to

the inner side and to the core, so that the core is contracted and made loose from the concrete.

For the purpose of explaining the invention 60 an example embodying the same has been shown in the accompanying drawing, in which the same reference characters have been used in all the views to indicate corresponding parts. In said drawing

65 Fig. 1, is a sectional elevation showing the core and the concrete applied thereto,

Fig. 2, is a detail sectional elevation showing the bottom part of the core and concrete 70 and a ring used for removing the set pipe from the core,

Fig. 3 is a diagrammatic sectional elevation showing the action of cooling of a tube being formed upon a conical form and upon a form having a projecting shoulder at the 75 larger end of the conical form respectively,

Fig. 4, is a somewhat diagrammatical elevation showing means for heating the concrete applied to the core,

Fig. 5, is a partial plan view of Fig. 4, 80 and

Fig. 6, is a detail sectional elevation showing a part of the core and the pipe on an enlarged scale.

85 In carrying out my improved process a solid and substantially cylindrical or slightly tapering core is used, which is vertically placed on a suitable rotary table, and which is slowly rotated about its vertical axis while flinging or squirting soft concrete thereon, 90 as has been described for example in my co-pending application for patent, Ser. No. 4,015. While in the method described in the said application a core is used which is made from several sectors, I use an integral 95 or solid hollow cylindrical or slightly tapering core  $a$ , by means of which a pipe is made which has a very smooth inner surface. At the end of larger diameter of the said core there is an enlarged annular portion  $a'$  the 100 outer diameter of which corresponds to the inner diameter of the usual enlarged portion of the pipes of this type used for making the pipe joint. Therefore the radius of the enlarged portion  $a'$  of the core exceeds the radius 105 of the adjacent portion of the body  $a$  of the pipe by the thickness of the wall of the complete concrete pipe plus the space required for applying the ordinary packing medium in the joint. It will be understood 110 that also the portion  $a'$  tapers slightly from the bottom end towards the body  $a$ , and that

the body  $a$  of the core slightly tapers from the bottom end to the top end thereof as shown in Fig. 1, the object of thus tapering the core being to facilitate the removing of 5 the core from the concrete pipe, as will be described hereinafter.

The core  $a, a'$  is made from strong and smooth material having high conductivity for heat. Preferably it consists of a suitable metal such as cast iron. But in some 10 cases I manufacture the same from concrete having metal chips embedded therein for increasing the conductivity for heat.

The pipe  $a, a'$  is closed at its top and 15 bottom ends by rigid lids  $b$  and  $b'$  made from metal such as cast iron, and the said lids are coated at one or both sides with layers  $c$  and  $c'$  made from a material of high insulating capacity such as rubber. In 20 some cases I place protective sheets  $c^o, c^o'$  of metal or other suitable material on the said layers of rubber. Preferably washers  $v$  and  $v'$  of rubber are placed between the end faces of the core  $a, a'$  and the lids 25  $b, b'$ .

Suitable means are provided for rigidly connecting the lids  $b$  and  $b'$  to the core  $a, a'$ . As shown in Fig. 1 a rod  $w$  is provided for this purpose. The lid  $b'$  is formed 30 at its bottom face with an axial cylindrical lug  $h$  adapted for engagement with a corresponding socket made in the rotary table, and the rod  $w$  is formed at its top end with an eye  $g$  for suspending the same from 35 the chain of a hoisting machine.

Through the upper lid  $b$  pipes  $k$  and  $k'$  are passed, through which a suitable heating or cooling medium may be circulated through the inner part of the core, and in 40 some cases I provide a vent  $x$  for removing the air from the core. The lower lid  $b'$  is formed with a discharge opening normally closed by a valve  $l$ , the stem  $l''$  being passed upwardly through the core and carrying at its outer end a nut  $l'$  for pressing the valve  $l$  on its seat.

At their outer sides the lids  $b$  and  $b'$  are provided with annular recesses  $b^o, b^o'$  having rings  $d$  and  $e$  fitted therein. The outer diameters of the said rings are equal 50 respectively to the outer diameter of the concrete pipe and the enlarged portion thereof, and they embrace respectively with their top and bottom parts the top and bottom parts of the core  $a, a'$ . Thus the outer portions of the said rings determine the thickness of the concrete pipe  $R$  and the position of the end faces of the said pipes. The rings  $d$  and  $e$  are connected with the 55 lids  $b$  and  $b'$  so that they may be readily removed therefrom. To show what may be done arms  $f$  are rockingly mounted on the lids, which arms are adapted to be turned outwardly for fixing the rings to the lids. 60 In Fig. 1 only one of the said arms is shown.

But I wish it to be understood that at least three arms are used for each ring  $d$  and  $e$ . When turning the said arms inwardly the rings  $d$  and  $e$  can be readily removed.

After constructing the core in the manner 70 described I place the same in vertical position on the rotary table and impart slow rotary movement thereto while gradually applying the soft concrete thereto. Apparatus suitable for this purpose has been described in my copending application for patent, Ser. No. 4,015 and I deem it not necessary to describe the apparatus in detail. The core may be placed on the said table while being at room temperature. But I prefer 80 slightly to heat the same, for example by shortly immersing the same into warm water, or filling the same with warm water. After the first part of the concrete has been applied the core is perfectly insulated as 85 against loss of heat, the lids being coated with insulating material in the manner described, and the concrete applied to the core  $a, a'$  having low conductivity for heat. The mass of concrete which is comparatively 90 cold, is uniformly and slightly heated from the core.

After moulding the inner layer of concrete having a thickness of one half the thickness of the desired wall of the pipe, 95 the said layer of concrete is allowed to set, and in order that the period of time required for setting be reduced I carry the core and the inner layer of concrete applied thereto into the apparatus shown in 100 Figs. 4 and 5, a suitable hoisting machine consisting of a crane  $K$  running on a suitable rail  $G$  being provided for this purpose. As shown the said apparatus consists of a pit comprising a large chamber  $A$  filled with 105 hot water and a plurality of small chambers  $B$ . The water contained in the chamber  $A$  is heated for example by means of a heating coil  $H$  to a temperature of from 40 to 60° C. The size of the chambers  $B$  is 110 comparatively small and it is not larger than is necessary for receiving the core  $a, a'$  and the concrete applied thereto. The chambers are heated by the heat transmitted therefrom to the chamber  $A$ . 115

After a pipe  $R$  and its core have been placed into one of the chambers  $B$  the lid  $F$  is closed. The small amount of air within the said chamber is rapidly saturated with vaporized water, and by reason of the elevated temperature the concrete begins to set after a short period of time. In this process only a very small amount of the water of the concrete is vaporized, so that no cracks are produced in the layer of concrete. After a 120 short period of time the concrete has set so far that it may be exposed to contact with warm water. Therefore, after removing the lid  $F$  the core is again elevated by the hoisting apparatus  $K$  and carried into the hot 125 130

water contained within the chamber A. Within the said water setting is completed within three or four hours. Thereafter the core and the set layer of concrete are carried to the flinging apparatus, where the second layer is applied to the inner layer in the same way as has been described above. If it is desired to manufacture re-inforced concrete pipes I apply the re-inforcing iron to the set inner layer prior to applying the outer layer thereto, the said re-inforcing iron being in the form of a net, a helically wound wire or strip iron. In Fig. 6 I have shown the core, the inner and outer layers and the re-inforcing iron on a larger scale, *a* being the core, *R'* the inner layer of concrete, *E* the helically wound strip iron, and *R''* the outer layer of concrete. In the said figure I have shown a very thin layer of concrete *R'*, which is first applied to the set inner layer *R'* before applying the strip iron *E* thereto, so that the said strip iron is wound into the said soft concrete and intimately connected with the said concrete. After applying the outer layer of concrete, the outer surface of the pipe indicated in Fig. 1 by the points *n*, *o*, *p*, *q*, may be moulded by removing the excess of material by cutting wires while gradually rotating the core. This method is known in the art and I deem it not necessary to describe the same in detail.

Now the core is again carried to the pit A, B, where the outer layer is made to set in the manner described above. Finally the core is removed from the pipe *R*.

After the core and the pipe carried thereby have been removed from the pit A the rings *d* and *e* are removed from the lids *b* and *b'*, and the core and mass of concrete *R* are placed with the bottom on the hinge *r* shown in Fig. 2, so that the whole mass of the core and pipe bears on the lower end face of the enlarged bottom part of the pipe. In order that the core be more readily placed on the said ring I prefer to form the lid with a bevelled margin *s*. Now the hot water which may be contained within the hollow of the core is discharged through the valve *l*, and a cooling medium, such as cold water is made to circulate through the said core. Thereby the core *a*, *a'* is slightly contracted while the concrete pipe *R* remains at elevated temperature by reason of its low conductivity for heat, so that it is not contracted. Therefore the core is made loose from the pipe.

Evidently the core is contracted not only in circumferential direction but also in axial direction. By reason of the shoulder *t* of the core the body *a* is contracted downwardly. The length of the pipe being about three meters, there is an appreciable longitudinal displacement of the core *a* relatively to the pipe *R*, which assists in disconnecting the

core from the pipe. I have found that ordinarily the core is automatically disconnected from the pipe, and that a slight blow made with a hammer is sufficient to remove the core from the pipe without injuring the latter. In order that the core be more readily separated from the pipe I provide the same with a very smooth surface, and in some cases I apply thereto a suitable medium such as oil, graphite or the like prior to applying the inner layer of concrete thereto.

It will be understood that in the manufacture of the pipes each core is used several hours for making a single pipe. Therefore, when using cores made from metal the cost of the stock of cores is very high. In order to reduce the cost I prefer to manufacture the cores from concrete having a high conductivity for heat, so that only the lids *b*, *b'* and the rings *d*, *e* are made from metal. In the practice of this part of my invention I manufacture a tubular mould from any suitable material, the inner configuration of which exactly corresponds to the inner form of the concrete pipe *R* and I place a core of metal or wood into the said pipe, which corresponds to the inner diameter of the core *a*, *a'*. The mould thus formed is filled with concrete having metal chips admixed thereto, and I allow the said concrete to set in the ordinary way. The concrete pipe *a*, *a'* which has thus been manufactured is used in the manner described above. Should the concrete core *a*, *a'* be injured after some time of use it may be replaced at low cost, while the lids *b*, *b'* and other metal parts may be used for any length of time.

The separation of the core from the concrete pipe may be further accelerated by externally heating the pipe *R* while internally cooling the core. For example, I place the core and pipe on the ring within a pit similar to A or within the pit A itself, so that the pipe is heated by the warm water contained within the said pit. Further, means may be provided for filling the chambers B with warm water after heating the pipe by means of air, and to return the hot water at the end of the setting process into the chamber A. When thus carrying out the process it is not necessary to carry the core from the chamber B into the chamber A. Apparatus for carrying out this modification of my method will readily suggest themselves to those skilled in the art, and I deem it not necessary to show the same in the drawings.

While in describing the invention reference has been made to particular examples embodying the same I wish it to be understood that I do not limit myself to the particular method and the apparatus described herein.

I claim:

1. The herein described method of manufacturing pipes from plastic matter, which

- consists in first moulding from the plastic matter a pipe, allowing the matter to set, coating the pipe with plastic matter, applying re-inforcing metal to the coat while still soft, thereafter applying another layer of plastic matter to the said re-inforcing metal and pipe, and allowing the said layer to set.
2. The herein described method of manufacturing pipes, which consists in applying plastic matter containing cement to a core, allowing the said plastic matter to set, applying a thin layer of the said plastic matter to the set matter, applying re-inforcing iron on the said thin layer while soft, applying another layer of the said plastic matter to the iron, and allowing the same to set, the thickness of the layers first and last applied being substantially equal to one half the thickness of the wall of the pipe to be made.
3. A mould for manufacturing pipes from plastic matter containing cement, comprising an integral tubular core, lids fixed to the end faces of said core and having a diameter equal to the outer diameter of said core, and rings fixed to said lids and formed with flanges embracing the ends of said core and having a diameter equal to the outer diameter of the pipe to be manufactured.
4. A mould for manufacturing pipes from plastic matter containing cement, comprising an integral tubular tapering core formed at the end of larger diameter with an enlarged annular portion, disks fixed to the end faces of said core and having diameters equal to the outer diameters of the adjacent portions of the core, and rings fixed to said lids and formed with flanges embracing the ends of the core and having outer diameters equal to the outer diameters of the adjacent portions of the pipe to be manufactured.
5. The herein described method of manufacturing pipes which consists in applying plastic matter containing cement to a core, allowing the said plastic matter to set, applying a thin layer of the said plastic matter to the set matter, applying re-inforcing helically wound flexible elongated iron on the said thin layer while soft, applying another layer of the said plastic matter to the iron, and allowing the same to set, the thickness of the layers first and last applied being substantially equal to one half the thickness of the wall of the pipe to be made.

In testimony whereof I have affixed my signature.

ALPHONS HORTEN.